

## UNITED STATES PATENT OFFICE

2,157,766

## BASIC LEAD NAPHTHENATE

Kenneth E. Long, South Euclid, Ohio, assignor to  
The Harshaw Chemical Company, Cleveland,  
Ohio, a corporation of Ohio

No Drawing. Application October 30, 1933,  
Serial No. 695,955

## 1 Claim. (Cl. 260—435)

This invention relates to lead compounds, and it is among the objects of the invention to provide an improvement in basic lead naphthenate.

To the accomplishment of the foregoing and related ends, the invention, then, comprises the features hereinafter fully described, and particularly pointed out in the claims, the following description setting forth in detail certain illustrative embodiments of the invention, these being 10 indicative however, of but a few of the various ways in which the principle of the invention may be employed.

Salts or soaps such as lead linoleate, oleate, naphthenate, etc., sold to the trade as such or under various trade names, are used in the paint, varnish, and printing ink industries as siccatives and are also used in grease making and in waterproofing compounds, etc. The usual commercial practice in preparation of these salts or soaps 15 consists of saponification of a fatty acid or its glyceride with alkali and precipitation of the lead soap with a soluble lead salt such as the acetate or nitrate. Another method consists of combining directly a lead compound, such as litharge, with a fatty acid, in a suitable kettle or container, with the aid of heat. This reaction is carried out at a temperature from 100° C. to 250° C. Water formed by the reaction is expelled at the time of formation as water vapor or steam. There is no great difference between the products made by either method with the exception that the fused products are usually darker in color and contain some free fatty acid, as it is difficult to bring into contact, in a fusion of this 25 type, every particle of litharge with the fatty acid. By either method the metallic content is at best substantially not higher than the acid combining equivalent.

In accordance with the present invention, a lead oxy-compound, viz., litharge, lead hydroxide or hydrated lead oxide is intimately mixed at a temperature below 100° C. with an organic acid of the fatty acid type which is water-insoluble or at least sparingly soluble. During this mixing a reaction takes place between the acid and the lead oxid with consequent formation of water. There is a rise in temperature of the reacting mass but conditions are controlled so that the heat generated is not sufficient to expel the water liberated by the reaction. In contradistinction to the general or old practice, I have found that by my method I can introduce litharge in amounts substantially in excess of the theoretical combining or molecular equivalent. I have 30 found also that all of the lead so introduced is

in chemical combination with the acid. As a further step, the temperature is raised to complete the reaction and drive off the water of reaction, or the water may be removed by any suitable means. 5

The mixing of the lead compound and acid must be positive and thorough to prevent formation of lumps of partially reacted material which are not easily incorporated if once formed. One effective way of thorough mixing is by grinding 10 the desired mixture of acid and lead compound on ink-grinding rolls.

The following examples are illustrative of the process:

I. 100 parts of naphthenic acid with an acid 15 value of about 250 are mixed with about 71 parts of litharge, being thoroughly incorporated, as on ink-grinding rolls, the temperature being maintained below 100° C. Reaction sets in readily and the disappearance of the litharge soon takes 20 place. With the substantial completion of the reaction, the temperature is raised to above 100° C., and less than 200° C., and water formed is driven off. The product is a lead soap containing approximately 40 per cent of lead. It is a soft, 25 gummy solid, soluble in mineral oil, naphtha, xylol, toluol, and oils such as linseed oil, etc.

II. 100 parts of synthetic fatty acids made by the oxidation of petroleum hydrocarbons and having an acid value of about 360, are mixed with 30 about 115 parts of lead oxide, PbO, with thorough incorporation, the temperature being maintained below 100° C. After thorough mixing, and progress of the reaction, the temperature may be raised to 100° C., or more, to remove the water 35 of reaction. The product is a basic lead salt containing approximately 52 per cent of lead. It is a waxy solid soluble in xylol, toluol, also oils such as linseed oil.

III. 60 parts of synthetic fatty acids made by 40 the oxidation of petroleum hydrocarbons and having an acid value of about 360, and about 40 parts of naphthenic acid with an acid value of about 250, are mixed with about 71 parts of lead oxide, PbO, as afore-described, the temperature 45 being maintained below about 100° C., and being finally raised thereabove to drive off water of reaction. The product is a basic lead salt containing approximately 40 per cent lead. It is a soft, pasty solid, readily soluble in solvents such as 50 above-enumerated.

IV. 100 parts of linseed oil fatty acid with an acid number of about 190, are mixed with about 71 parts of lead oxide, PbO, for instance by grinding on rolls, to a smooth paste at ordinary 55

temperature. The temperature is then slowly raised to about 100° C., and the reaction is completed, and the temperature is then further raised to about 180° C. to drive off water.

5 Other organic acids can similarly be reacted, such as fatty oil acids such as of linseed oil, fish oil, soy bean oil, corn oil, tung oil, etc. Where dealing with acids of rather high molecular weight, the reaction may be started particularly 10 advantageously by the presence of a small or catalytic amount of water. For instance, by moistening the litharge or the like with water as it is mixed with the acid, or by adding a small quantity of water to the mixture. On addition 15 of the water, the reaction promptly starts. In most cases, and particularly with lower molecular weight fatty acids, reaction sets in without addition of water, and water is in fact formed in the reaction. By maintaining the temperature 20 carefully below 100° C., the advantageous

progress of reaction is had, as already noted, and the temperature is to be raised ultimately, more particularly for the purpose of driving off water.

Other modes of applying the principle of the invention may be employed, change being made 5 as regards the details described, provided the features stated in any of the following claims, or the equivalent of such, be employed.

I therefore particularly point out and distinctly 10 claim as my invention:—

A lead salt product of naphthenic acid containing combined lead to the extent of more than one combining equivalent weight of lead to each combining equivalent weight of acid but not substantially over such proportion as involved in 15 a ratio of about 71 parts of PbO to 100 parts of naphthenic acid of acid value about 250, and being thereby basic but below maximum possible basicity.

KENNETH E. LONG. 20